

## [54] CORROSION RESISTANT AUSTENITIC STEEL

[75] Inventor: **Albert G. Hartline, III;**  
Brackenridge, Pa.[73] Assignee: **Allegheny Ludlum Industries, Inc.,**  
Pittsburgh, Pa.[22] Filed: **Oct. 4, 1973**[21] Appl. No.: **403,347**[52] U.S. Cl. .... **75/122, 75/126 B, 75/126 J,**  
**75/129**[51] Int. Cl. .... **C22c 39/14, C22c 33/00**[58] Field of Search ..... **75/122, 126 B, 129**

## [56] References Cited

## UNITED STATES PATENTS

|           |        |                |          |
|-----------|--------|----------------|----------|
| 2,949,355 | 8/1960 | Dyrkacz .....  | 75/126 B |
| 3,029,171 | 4/1962 | Rostoker ..... | 75/126 B |
| 3,556,777 | 1/1971 | Petry .....    | 75/126 B |

Primary Examiner—Hyland Bizot  
Attorney, Agent, or Firm—Vincent G. Gioia; Robert F. Dropkin

## [57] ABSTRACT

A substantially non-porous, austenitic stainless steel that is resistant to dilute sulfuric acid and to chloride pitting, and a method of making it, are disclosed. The steel includes from 21–45 percent manganese, from 10–30 percent chromium, from 1–5 percent molybdenum, from 0.85–3 percent nitrogen, up to 2 percent silicon, up to 1 percent carbon and the balance iron and residuals. In addition to containing elements within the above-noted composition ranges, the alloys must be such that:

$$1. \%Cr + \%Mo + 0.8(\%Mn) - 11.8(\%N) - 0.1(\geq 28.5)$$

$$2. 30(\%C + \%N) + 0.5 (\%Mn)/\%Cr + \%Mo + 1.5 (\%Si) \geq 1.5$$

The steels are cast and worked to avoid a dwell period in the temperature range 1,000–1,600°F.

8 Claims, 1 Drawing Figure



PATENTED NOV 12 1974

3,847,599



## CORROSION RESISTANT AUSTENITIC STEEL

## BACKGROUND OF THE INVENTION

Corrosion resistant steels, known as stainless steels, have long been known and are presently available with a variety of properties. Austenitic stainless steels, which are those consisting substantially of a single austenite phase, possess the best properties of corrosion resistance and good mechanical properties, particularly at high temperature. Austenitic stainless steels in the past have been steels in which chromium and nickel are the principal alloying agents. However, nickel is not an abundant metal and the increased demand for it has increased its price and made its supply uncertain, particularly in critical times. Substitutes for nickel in the chromium-nickel austenitic stainless steels have long been sought. Recently the combined use of manganese, nitrogen and chromium in carefully balanced amounts has produced an austenitic stainless steel. This steel is described in U.S. Pat. application Ser. No. 251,637, filed May 8, 1972; and although it is an excellent steel, it is somewhat subject to attack by sulfuric acid and chloride environments.

## SUMMARY OF THE INVENTION

The present invention is a chromium-manganese-molybdenum-nitrogen steel that is substantially non-porous, austenitic and highly resistant to attack by sulfuric acid and chloride environments. The alloy of this invention contains from 21-45 percent manganese, from 10-30 percent chromium, from 1-5 percent molybdenum, from 0.85-3 percent nitrogen, up to 2 percent silicon, up to 1 percent carbon and the balance iron and residuals. All compositions in this specification and the following claims are in percent by weight of the total composition unless otherwise specified.

In addition to the foregoing ranges, the composition of the alloys must be balanced in accordance with the following equations:

$$1. \%Cr + \%Mo + 0.8(\%Mn) - 11.8(\%N - 0.1) \geq 28.5$$

$$2. 30(\%C + \%N) + 0.5(\%Mn)/\%Cr + \%Mo + 1.5(\%Si) \geq 1.5$$

In the alloys of the present invention, chromium must be present to produce the same effect that it does in prior art alloys. The alloys of this invention must contain from 10-30 percent chromium. At least 10 percent 2 is required to give the steel its outstanding corrosion resistance. Chromium also has a secondary effect upon the strength of the steel and is a primary element in increasing the steel's solubility for nitrogen. An upper limit of 30 percent chromium is imposed as chromium is a ferrite former and excessive amounts of ferrite might form with higher chromium levels and in turn degrade the properties of the steel. A preferred chromium content is in the range of 15-27 percent in that steels containing this range of chromium are easy to process while still having good corrosion resistance and strength.

The manganese in the alloy of this invention is present in amounts of from 21-45 percent. Since manganese is an austenitizer and increases the solubility of nitrogen in the steel, amounts in excess of 21 percent are required. An upper limit of 45 percent, and preferably an upper limit of 30 percent, manganese is imposed for economic considerations and because manganese tends to attack furnace refractories.

Nitrogen, a strong austenitizer, should be present in the steel in amounts of from 0.85-3 percent. At least 0.85 percent is required for its austenitizing effect and because it is the primary strengthening element of the steel. Amounts of nitrogen in excess of 3 percent tend to yield porous ingots which are not satisfactory. The nitrogen content of the alloy of this invention preferably is from 1.05-1.5 percent.

The molybdenum content of the alloy of this invention must be between 1-5 percent. Although molybdenum has been known as an alloy additive in the past, in the present invention the molybdenum may be employed to reduce the amount of chromium and manganese employed, may be employed to increase the solubility of nitrogen, and most importantly reduces the susceptibility of the resultant alloy to attack by dilute sulfuric acid and to pitting attack by chlorides. The molybdenum-containing alloy of this invention is as strong or stronger than the above referred to chromium-manganese-nitrogen alloys.

Carbon, of course, is a well-known austenitizer and strengthener for steels and is employed in the alloys of this invention in amounts up to 1 percent. The concentration of carbon must be maintained below that level in that larger amounts can remove chromium from solid solution by combining with it to form chromium carbides and because carbon can reduce the solubility of the steel for nitrogen by occupying interstitial sites normally filled with nitrogen. It is preferred that less than 0.15 percent carbon be present in the alloy of this invention. Higher carbon contents require higher annealing temperatures to put carbides into solution.

The alloys of the present invention may tolerate silicon concentrations as high as 2 percent but preferably the silicon is below 1 percent. Higher quantities of silicon tend to remove manganese from the alloy in the form of manganese silicates and tend to form inclusions in the steel.

Although the residuals in the iron need not be identified and do not significantly affect the properties of the alloy, the usual residuals may be identified as phosphorus, sulfur, tungsten, cobalt and nickel.

Since the stainless steel composition of this invention is desirably a substantially one-phase austenitic material, thermal treatments that tend to precipitate other phases should be avoided. Although the alloys of this invention are not particularly sensitive to precipitation of other phases, the method of preparation employed should avoid long dwell periods in the 1,000-1,600°F temperature range. Long dwell periods would be characterized by furnace cooling. For ordinary thicknesses air cooling or quenching are sufficient to carry the alloy through the 1,000-1,600°F range quickly enough to avoid precipitation of detrimental phases such as sigma phase.

## DETAILED DESCRIPTION OF THE INVENTION

The accompanying drawing illustrates two plots of the 1.0 percent nitrogen section of the iron-chromium-manganese-nitrogen quaternary phase diagram. One plot illustrates that section wherein the alloy contains only residual amounts of molybdenum while the molybdenum plot illustrates that section containing 3 percent molybdenum.

As indicated in equations (1) and (2) set forth above, molybdenum has a significant effect both on the austenitic structure of the alloy and on the ability of the

alloy to maintain nitrogen in solution both in the liquid phase and in the resultant solid phase. Molybdenum within the composition limits set forth herein appears to be a replacement for chromium in that the combined molybdenum-chromium composition of the alloys determines where a two-phase austenite-ferrite alloy structure begins as compared with a single phase austenite structure, as well as where nitrogen precipitates from solution causing ingot porosity. In the drawing the area above line 1—A and 1'—A' generally represents compositions where a two-phase alloy of austenite and ferrite exists. As mentioned above, this two-phase system is undesirable because it does not have the good mechanical or chemical properties of a single-phase austenitic alloy. The area below the lines 1—A and 1'—A' are single-phase austenitic alloys.

Equation (2) defines the lines 2—B and 2'—B'. The area below these lines represents compositions where nitrogen comes out of solution during solidification and creates porous ingots. The areas above the lines 2—B and 2'—B' is where nitrogen remains in solution during solidification and non-porous ingots are formed.

The areas A—C—B and A'—C'—B' therefor represent the areas in which the alloys of this invention and of the prior art fall for this particular cross section of the quaternary phase diagrams illustrated. The alloys of the present invention fall in the area A—C—B. It may be noted that a single-phase alloy having no porosity may be obtained with substantially less chromium and with substantially less manganese in accordance with the present invention.

To demonstrate the benefits of this invention, four alloys were prepared having compositions set forth in Table I.

TABLE I

| Element | % Weight |         |         |         |
|---------|----------|---------|---------|---------|
|         | Alloy 1  | Alloy 2 | Alloy 3 | Alloy 4 |
| Mn      | 30.40    | 29.98   | 30.39   | 30.39   |
| Cr      | 20.45    | 20.34   | 19.97   | 20.02   |
| Mo      | 0.033    | 1.02    | 1.96    | 2.95    |
| N       | 1.00     | 1.18    | 1.18    | 1.18    |
| Ni      | 0.26     | 0.23    | 0.24    | 0.24    |
| Cu      | 0.20     | 0.16    | 0.16    | 0.16    |
| Si      | 0.48     | 0.40    | 0.36    | 0.42    |
| C       | 0.092    | 0.062   | 0.062   | 0.064   |
| S       | 0.009    | 0.010   | 0.011   | 0.011   |
| P       | 0.014    | 0.008   | 0.008   | 0.008   |

The alloys of Table I are substantially the same alloys with the exception of the molybdenum content. In effect, the alloys are all nominally 30 percent manganese, 20 percent chromium, 1 percent nitrogen alloys containing respectively a residual amount, 1, 2 and 3 percent molybdenum.

The alloys described in Table I were all prepared in the same way. All alloys were prepared from melted materials in an air induction furnace and were composed of commercial grades of ferroalloys and pure elements. The heats were cast from approximately 2,650°F into 35 pound cast iron ingot molds. After solidification, the ingots were examined for porosity which was not observed in any of the alloys. The hot processing of the alloys consisted of grinding to remove casting imperfections, heating the ingots at 2,250°F for an appropriate amount of time, and hot rolling to the desired width and thickness. While the hot strength appeared to increase with the addition of molybdenum, the ingots were rolled without incident. The hot rolled materials were annealed at 1,950°F on a schedule of 120 minutes per inch of material thickness, subsequently blasted and pickled in a mixture of 15 percent nitric acid and 3 percent hydrofluoric acid, cold rolled 50 percent to further homogenize the structure, final annealed at 1,950°F on the same schedule as mentioned above and again pickled. At various stages of the processing, samples were obtained to determine the mechanical properties of the metals. These properties are set forth in Table II. The strength data were obtained after annealing for 7 minutes at 1,950°F because this treatment produces a condition of minimum strength and maximum ductility in all alloys so that truly comparative data are obtained. It may be noted that the addition of molybdenum does not have a significant effect upon the mechanical properties of a nominal 20 percent chromium-30 percent manganese-1 percent nitrogen stainless steel.

The alloys of this invention are resistant to pitting attack in chloride environments. The resistance to pitting attack was measured in a crevice corrosion test wherein standardized specimens of the various alloys are immersed in 10% ferric chloride solution for 72 hours. The pitting attack is measured by the mean weight loss of a number of samples of each alloy. The

TABLE II

| Tensile Strength<br>As Annealed | Alloy Number    |                 |                 |                 |
|---------------------------------|-----------------|-----------------|-----------------|-----------------|
|                                 | 1               | 2               | 3               | 4               |
| 0.2% Yield Strength (KSI)       |                 |                 |                 |                 |
| Longitudinal                    | 97.5—<br>99.2   | 105.9—<br>109.1 | 108.4—<br>109.6 | 108.9—<br>109.3 |
| Transverse                      | 98.2—<br>100.5  | 105.8—<br>107.7 | —               | 109.4           |
| Ultimate Tensile Strength (KSI) |                 |                 |                 |                 |
| Longitudinal                    | 146.1—          | 151.6—          | 156.5—          | 154.9—          |
| Transverse                      | 147.7—<br>149.2 | 155.2—<br>155.7 | —               | 157.8           |
| Elongation (%)                  |                 |                 |                 |                 |
| Longitudinal                    | 50-52           | 48-52           | 49-51           | 50-51           |
| Transverse                      | 45-50           | 49-50           | —               | 50              |
| Hardness (Rockwell)             | 28              | 29              | 28.5            | 29              |

resistance of the alloys of the present invention to chloride pitting are set forth in Table III.

TABLE III

| Alloy Number          | 1     | 2     | 3     | 4    |
|-----------------------|-------|-------|-------|------|
| Mo Content (%)        | 0.033 | 1.02  | 1.96  | 2.95 |
| Mean Wt. Loss (grams) | 1.101 | 0.060 | 0.003 | 0    |

The potentiokinetic technique is another method for measuring the pitting resistance of an alloy to chloride solutions. In this technique an alloy specimen is placed in contact with an appropriate chloride solution and an electrical potential is imposed on the specimen at increasing voltages until a breakthrough point at which a surge of current passes through the solution. Higher breakthrough potentials indicate greater resistance to chloride pitting. A significant aspect of the potentiokinetic technique is that the ability of an alloy to self-passivate may be found by reversing the potential to determine where a high resistance to current flow is obtained after the breakthrough. Alloys with a tendency to self-passivate display a decrease in current at a voltage near the breakthrough potential. Alloys 2, 3 and 4 all showed better resistance to chloride pitting in potentiokinetic tests than did alloy 1. Of equal significance is that alloys 2, 3 and 4 all showed better self-passivation properties when the potential on the specimen was reduced than did alloy 1.

The specimens of alloys 1 through 4 inclusive were also subjected to standard corrosion testing to measure their resistance to sulfuric acid. Resistance of an alloy to sulfuric acid is measured by exposing an alloy specimen to sulfuric acid and obtaining the anodic polarization data and the cathodic polarization data and determining their intersection point on a plot of voltage versus current. A correlation is known to exist between the intersection points of these lines and the resistance of the specimen to sulfuric acid corrosion. Intersection of these lines at lower current flows indicates better resistance to sulfuric acid. Table IV contains data obtained in the foregoing test on specimens of alloys 1 through

It may be noted from Table IV that even the smallest amount of molybdenum in the alloy of this invention significantly increases the resistance of the alloy to sulfuric acid corrosion.

5. What is claimed is:

1. An alloy consisting essentially of about 21-45 percent manganese, about 10-30 percent chromium, about 1-5 percent molybdenum, about 0.85-3 percent nitrogen, up to 1 percent carbon, up to 2 percent silicon and the balance iron and residuals wherein the composition is such that:

$$1. \%Cr + \%Mo + 0.8(\%Mn) - 11.8(\%N - 0.1) \geq 28.5$$

$$2. 30(\%C + \%N) + 0.5(\%Mn)/\%Cr + \%Mo + 1.5(\%Si) \geq 1.5$$

2. The alloy in accordance with claim 1 comprising from about 1-3 percent molybdenum.

3. An alloy in accordance with claim 1 comprising 21-30 percent manganese.

4. An alloy in accordance with claim 1 comprising 15-27 percent chromium.

5. An alloy in accordance with claim 1 comprising 1.05-1.5 percent nitrogen.

6. An alloy in accordance with claim 1 comprising 0-0.15 percent carbon.

7. An alloy in accordance with claim 1 comprising 0-1.0 percent silicon.

8. A method for producing a substantially non-porous austenitic stainless steel which comprises comprising an alloy containing about 21-45 percent manganese, about 10-30 percent chromium, about 1-5 percent molybdenum, about 0.85-3 percent nitrogen, up to 1 percent carbon, up to 2 percent silicon, and the balance iron and residuals, wherein the composition is such that:

$$1. \%Cr + \%Mo + 0.8(\%Mn) - 11.8(\%N - 0.1) \geq 28.5$$

$$2. 30(\%C + \%N) + 0.5(\%Mn)/\%Cr + \%Mo + 1.5(\%Si) \geq 1.5$$

TABLE IV

| Anodic-cathodic Polarization                                                      | Alloy 1 | Alloy 2 | Alloy 3 | Alloy 4 |
|-----------------------------------------------------------------------------------|---------|---------|---------|---------|
| 1. 0N H <sub>2</sub> SO <sub>4</sub> intersection at (milli-amp/cm <sup>2</sup> ) | 4.0     | 0.002   | 0.002   | 0.002   |
| 5. 0N H <sub>2</sub> SO <sub>4</sub> intersection at (milli-amp/cm <sup>2</sup> ) | —       | —       | —       | 0.0014  |

4. The resistance to sulfuric acid for all specimens was measured at 1.0 normal concentration and the resistance of alloy 4 containing nominally 3% molybdenum was also measured at 5.0 normal sulfuric acid.

55 melting said materials to form a homogeneous liquid phase and solidifying the resultant liquid phase without a dwell period in the temperature range from about 1,000°-1,600°F.

\* \* \* \* \*

UNITED STATES PATENT OFFICE  
CERTIFICATE OF CORRECTION

PATENT NO. : 3,847,599

DATED : November 12, 1974

INVENTOR(S) : Albert G. Hartline, III

It is certified that error appears in the above-identified patent and that said Letters Patent are hereby corrected as shown below:

1. Within the abstract, equation 1 contains an improperly typed parenthesis in the term 11.8(%N - 0.1).
2. Within the abstract - equation 2, and in column 1, line 43 and column 6, lines 15 and 40, equation 2 is somewhat misleading in that the structure of this fraction would appear to contain only a Mn to Cr ratio. The equation should read:

$$[30\%C + \%N] + 0.5(\%Mn) \geq 1.5$$

3. Column 1, line 48, "At least 10% 2 is required ..." This should read, "At least 10% chromium is required ..."

Signed and sealed this 15th day of July 1975.

(SEAL)

Attest:

RUTH C. MASON  
Attesting Officer

C. MARSHALL DANN  
Commissioner of Patents  
and Trademarks

UNITED STATES PATENT OFFICE  
CERTIFICATE OF CORRECTION

PATENT NO. : 3,847,599  
DATED : November 12, 1974  
INVENTOR(S) : Albert G. Hartline III

It is certified that error appears in the above-identified patent and that said Letters Patent are hereby corrected as shown below:

Within the abstract, equation 1 contains an improperly typed parenthesis in the term 11.8(%N - 0.1).

Within the abstract - equation 2, and in column 1, line 43 and column 6, lines 15 and 40, equation 2 is somewhat misleading in that the structure of this fraction would appear to contain only a Mn to Cr ratio. The equation should read:

$$[30(\%C + \%N) + 0.5(\%Mn)] / [\%Cr + \%Mo + 1.5(\%Si)] > 1.5$$

Column 1, line 48, "At least 10% 2 is required..."  
This should read, "At least 10% chromium is required..."

Signed and Sealed this

fifth Day of July 1977

[SEAL]

Attest:

RUTH C. MASON  
Attesting Officer

C. MARSHALL DANN  
Commissioner of Patents and Trademarks